

## 1

2,980,641

**SOLUTIONS OF POLYPYRROLIDONE IN AQUEOUS PHYTIC ACID AND PROCESS FOR MAKING SAME**

Paul R. Cox, Jr., Decatur, Ala., assignor to The Chemstrand Corporation, Decatur, Ala., a corporation of Delaware

No Drawing. Filed Sept. 25, 1958, Ser. No. 763,198

15 Claims. (Cl. 260—29.2)

This invention relates to new compositions of matter. More particularly, the invention relates to new compositions of matter comprising polypyrrolidone and solvents therefor.

Polypyrrolidone possesses many excellent properties which make it desirable for utilization in the manufacture of end products, such as ribbons, films, fibers, filaments, rods, bristles, lacquers, coatings, shaped articles and the like. Polypyrrolidone can be converted into shaped articles in many ways. For example, it may be cast into films or forced through multi-hole spinnerets to form fibers or filaments. Regardless of the end use to which the polypyrrolidone is to be put, it is generally more convenient and efficient to employ the polymer in a solution. This is well illustrated in the textile industry where polypyrrolidone is employed in the formation of fibers and filaments, which are manufactured by several methods of spinning, such as melt spinning, dry spinning, and wet spinning.

In the melt spinning method, the polymer is heated to a high temperature until it becomes molten and is thereafter forced through sand packs and the like, and thence through a spinneret from which it is extruded in filamentary form. This method has, however, many disadvantages, although it is widely used in the industry at the present time in the production of synthetic fibers and filaments. The high temperatures used in melt spinning require the exercise of extreme care in order to prevent decomposition of the polymer. Furthermore, the high temperatures also affect the chemical and physical characteristics of the polymer and thereby result in a product of inferior quality. In addition to these disadvantages, it is extremely difficult to add to the molten polymer at such high temperatures compounds such as dyes, anti-static agents, plasticizers and the like.

In the dry spinning method of fiber formation, the polymer is dissolved in a suitable solvent and subsequently extruded from a spinneret into a heated atmosphere in order to evaporate the polymer. Even this method, however, has its disadvantages, since during the period of time in which the solvent evaporates, considerable damage may be inflicted on the fibers because of the high heat necessary to bring about solvent evaporation. Another disadvantage of the dry spinning method, and of the melt spinning method also, is the added cost necessary to maintain such high temperatures needed to manufacture the desired end product.

The wet spinning method obviates many of the disadvantages of both melt spinning and dry spinning. In order to form filaments by the wet spinning method, the polymer is dissolved in a suitable solvent and extruded from a spinneret into a coagulating bath capable of leaching the solvent from the fiber. Normally, this method may be carried out at temperatures much lower than either the melt spinning or dry spinning methods. If it is desired to use additives, such as dyes, anti-static agents, fire-retarding agents, plasticizers and the like, in the polymeric solution, they may be incorporated therein

## 2

without the danger of decomposition or seriously affecting the properties of the end product where the wet spinning method of filamentary formation is employed. Furthermore, it is much easier to introduce such additives into a solution than to introduce them into a molten composition. Then again, solutions are much easier to handle during processing, and in many cases may be stored for long periods of time without a change in physical and chemical properties. It is much easier to cast a film from a solution than to cast it from a molten composition. It is readily apparent, therefore, that solutions of polypyrrolidone present many distinct advantages over molten compositions in the manufacture of end products.

Accordingly, it is a primary object of the present invention to provide new and useful compositions of matter comprising polypyrrolidone. It is another object of the invention to provide solutions of polypyrrolidone. It is a further object of the invention to provide solutions of polypyrrolidone which may be converted into shaped articles, such as ribbons, films, filaments, fibers, rods, bristles, lacquers, coatings and the like. It is still another object of the invention to provide a process for the preparation of polypyrrolidone solutions. Other objects and advantages of the instant invention will be readily apparent from the description thereof which follows hereafter.

In general, the objects of the present invention are accomplished by dissolving polypyrrolidone in aqueous phytic acid or aqueous solutions of the water-soluble alkali metal acid salts, alkaline earth metal acid salts or the mixed alkali and alkaline earth metal acid salts thereof.

The phytic acid compounds utilized in the practice of this invention are normally employed in aqueous solutions. The water is generally present in a range of 5 to 50 percent, based on the total weight of the solvent. However, less than 5 percent or more than 50 percent water may be employed with consequent loss of solvent power and in such cases the water and phytic acid mixture is an excellent plasticizer for polypyrrolidone. It is preferred, however, that the water be employed in a range of 30 to 50 percent, based on the total weight of the solvent.

In addition to the phytic acid itself, the water-soluble alkali metal acid salts, alkaline earth metal acid salts and the mixed acid salts of the alkali metals and alkaline earth metals of phytic acid which are useful as solvents in this invention include lithium acid phytate, potassium acid phytate, sodium acid phytate, strontium acid phytate, calcium acid phytate, magnesium acid phytate, lithium calcium acid phytate, sodium magnesium acid phytate, sodium potassium acid phytate, lithium strontium acid phytate, lithium potassium acid phytate, lithium sodium acid phytate, lithium magnesium acid phytate, potassium strontium acid phytate, potassium calcium acid phytate, sodium strontium acid phytate, sodium calcium acid phytate, calcium strontium acid phytate, magnesium strontium acid phytate, calcium magnesium acid phytate, and the like.

Polypyrrolidone soluble in the solvents of this invention may be prepared by various processes. Generally, however, polymeric pyrrolidone is prepared by polymerizing monomeric pyrrolidone in the presence of a catalyst or a catalyst and activator at temperatures in the range of  $-70^{\circ}\text{C}$ . to  $100^{\circ}\text{C}$ . However, since the polymerization reaction proceeds well in the range  $20^{\circ}\text{C}$ . and  $70^{\circ}\text{C}$ ., these temperatures are preferred in carrying out a polymerization procedure.

In the preparation of polypyrrolidone, a large number of known catalysts are available to catalyze the polymerization. Among such catalysts, there may be named the alkali metals, namely, sodium, potassium and lithium,

as well as the hydrides, hydroxides, oxides and salts of the alkali metals, that is, such salts as sodium, lithium and potassium pyrrolidone. Organic metallic compounds, preferably those which are strongly basic, may also be used as catalysts. Examples of such compounds are lithium, potassium and sodium alkyls and aryls of the alkali metals, such as sodium phenyl. Another suitable catalyst is sodium amide. The alkali hydrides, however, are the preferred catalysts, since a distinct advantage is obtained by their use. Sodium hydride, for example, does not react in the polymerization mixture to form water which, as is well known, has a deleterious effect upon pyrrolidone polymerization. Where a water-forming catalyst, such as sodium hydroxide, is employed as a catalyst, all water of reaction must be removed from the reaction mixture by vacuum distillation or other means in order to promote polymerization. Generally, the catalyst may be employed in a range of 0.002 to 0.25 chemical equivalents based upon one mole of monomeric pyrrolidone in carrying out a polymerization reaction.

Although polypyrrrolidone having acceptable properties can be prepared by using a catalyst alone, it is preferable to employ an activator in conjunction with any of the catalysts mentioned above, since the polymer prepared in the presence of both a catalyst and activator has greatly improved properties over polypyrrrolidone prepared in the presence of a catalyst alone. Among the compounds which may be employed as activators, there may be named the acyl compounds, such as acetyl pyrrolidone, acetyl morpholone, and the like; lactones, such as gamma butyrolactone, and the like; alkyl esters of mono- and dicarboxylic acids, such as ethyl acetate, ethyl oxalate, and the like; the esters of polyhydric alcohols such as ethylene glycol diacetate, and the like; and nitrogen dioxide and organic nitrites having the general formula:



wherein R is selected from the group consisting of alkyl groups containing 1 to 10 carbon atoms, haloalkyl groups containing 2 to 10 carbon atoms, nitroalkyl groups containing 2 to 10 carbon atoms, aralkyl groups containing 7 to 10 carbon atoms, and alkoxy alkyl groups containing 3 to 12 carbon atoms. Among the nitrites falling into the general formula set out above, there are methyl nitrite, ethyl nitrite, n-propyl nitrite, iso-propyl nitrite, n-butyl nitrite, iso-butyl nitrite, amyl nitrite, iso-amyl nitrite, hexyl nitrite, heptyl nitrite, octyl nitrite, nonyl nitrite, decyl nitrite, and their isomeric forms, and the like; haloalkyl nitrites such as 2,2,2-trichloroethyl nitrite; the dihaloalkyl nitrites, such as 2,2-dichloroethyl nitrite, 2,2-dichloropropyl nitrite, 2,2-dichlorobutyl nitrite, 2,2-dichloroamyl nitrite, 2,2-dichlorohexyl nitrite, 2,2-dichloroheptyl nitrite, 2,2-dichlorooctyl nitrite, 2,2-dichlorononyl nitrite, 2,2-dichlorodecyl nitrite, and the like; monochloroalkyl nitrites, their isomeric forms, and the like; nitroalkyl nitrites, such as 2-nitroethyl nitrite, 2-nitropropyl nitrite, 2-nitrobutyl nitrite, 2-nitroamyl nitrite, 2-nitrohexyl nitrite, 2-nitroheptyl nitrite, 2-nitrooctyl nitrite, 2-nitrononyl nitrite, 2-nitrodecyl nitrite, and their isomeric forms, and the like; aralkyl nitrites, such as benzyl nitrite, 2-methylbenzyl nitrite, 3-methylbenzyl nitrite, 4-methylbenzyl nitrite, 2-ethylbenzyl nitrite, 3-ethylbenzyl nitrite, 4-ethylbenzyl nitrite, 2-propylbenzyl nitrite, 3-propylbenzyl nitrite, 4-propylbenzyl nitrite, 2-methyl-3-ethylbenzyl nitrite, 2-methyl-4-ethylbenzyl nitrite, 2-methyl-5-ethylbenzyl nitrite, 2-methyl-6-ethylbenzyl nitrite, 3-methyl-4-ethylbenzyl nitrite, 3-methyl-5-ethylbenzyl nitrite, 3-methyl-6-ethylbenzyl nitrite, 4-methyl-2-ethylbenzyl nitrite, 4-methyl-3-ethylbenzyl nitrite, 2,3-dimethylbenzyl nitrite, 2,4-dimethylbenzyl nitrite, 2,5-dimethylbenzyl nitrite, 2,6-dimethylbenzyl nitrite, 3,4-dimethylbenzyl nitrite, 3,5-dimethylbenzyl nitrite, and the like; and alkoxyalkyl nitrites, such as 2-methoxyethyl nitrite, 2-ethoxyethyl nitrite, 2-propoxyethyl nitrite, 2-butoxyethyl nitrite, 2-pentoxyethyl nitrite, 2-hexaoxyethyl nitrite,

2-heptoxyethyl nitrite, 2-octoxyethyl nitrite, 2-nonoxyethyl nitrite, 2-deoxyethyl nitrite, and their isomeric forms, and the like.

Another excellent polymerization activator is carbon disulfide. Silicon halides and organic silicon halides having the general formula:



wherein R is a saturated or unsaturated aliphatic or aromatic hydrocarbon radical containing 1 to 10 carbon atoms, a saturated or unsaturated aliphatic or aromatic halogenated hydrocarbon radicals containing 1 to 18 carbon atoms, and X is a halogen, z is an integer from 1 to 4 inclusive, and y is equal to 4-z, wherein R may be similar or dissimilar radicals, may also be employed to activate polymerization of pyrrolidone. Among the silicon halides and organic silicon halides there may be named tetrachlorosilane,  $\alpha,\beta$ -dichloroethyltrichlorosilane, bis(chloromethyl)methylchlorosilane, butyltrichlorosilane, chloromethylmethyldichlorosilane, dichloromethyl-dimethylchlorosilane, diethyldichlorosilane, dimethyldichlorosilane, diphenyldichlorosilane, ethyltrichlorosilane, methyltrichlorosilane, phenyltrichlorosilane, propyltrichlorosilane, trimethylchlorosilane, vinyltrichlorosilane, the iodo- and bromo-forms of the above compounds, and many others. The trihalides of phosphorous, aluminum, bismuth and antimony, the tetrahalides of titanium, tin, zirconium and lead, and the pentahalides of antimony and phosphorous are also useful as activators in the polymerization of pyrrolidone. Such compounds include aluminum trichloride, aluminum tribromide, aluminum triiodide, stannic tetrachloride, stannic tetrabromide, lead tetrachloride, zirconium tetrachloride, bismuth trichloride, bismuth tribromide, antimony trichloride, antimony tribromide, antimony triiodide, antimony pentachloride, antimony pentaiodide, antimony pentafluoride, and the like. The phosphorous halides include phosphorous tribromide, phosphorous pentabromide, phosphorous trichloride, phosphorous pentachloride, phosphorous trifluoride, phosphorous pentafluoride, phosphorous triiodide, and the like. Generally, in the preparation of polypyrrrolidone wherein both a catalyst and activator are employed to bring about polymerization, the activator is utilized in a range of 0.0001 to 0.075 chemical equivalents of activator, based upon one mole of monomeric pyrrolidone.

The polypyrrrolidone soluble in the solvents of this invention is prepared by simple polymerization methods. It can be prepared readily by well-known solution, emulsion, suspension or bulk polymerization procedures. The solution and emulsion polymerizations may be either batch, semi-continuous or continuous methods. When solution polymerization is employed, the monomer is dissolved in a solvent such as 1,4-dioxane, the desired catalyst or activator, or both, added to the solution and the polymerization carried out under the proper conditions. Well-known solution polymerization apparatus is suitable for preparing the polypyrrrolidones described herein. Where either emulsion or suspension polymerization techniques are employed to prepare the polymer, the monomer containing the catalyst is dispersed in a known solvent, such as petroleum ether, and an emulsifying agent then added to the dispersion. Subsequently, the desired activator is injected into the mixture and the dispersion is polymerized until the reaction is complete. At this time, suitable coagulant is added to the polymerization mixture in order to precipitate the polymer. A suitable emulsifying agent is sodium lauryl sulfate, and a suitable coagulant is phosphorous acid. When batch polymerization methods are employed in preparing polypyrrrolidone, no diluent is necessary.

Polypyrrrolidone prepared in accordance with the procedures set forth hereinabove has a melting point of about 260° C. and a specific viscosity of from about 0.3 to 4.5 or more. It is thus particularly adapted for the manu-

facture of shaped articles such as filaments, fibers, films, rods, bristles, and the like. Lower molecular weight polymers prepared in the same manner are suitable for the preparation of coatings or lacquers.

When dissolving polypyrrolidone in the solvents of the present invention, it may be employed in varying concentrations. The concentration of the polymer in the solvent depends upon the nature of the polymer, the solvent employed and the temperature, which in turn affect the viscosity of the solution. Normally, when the solution is to be employed in the manufacture of fibers and filaments, as much as 50 percent of the polymer, based on the total weight of the solution, may be dissolved in the phytic acid solvents. While it is preferred to employ 20 to 40 percent, based on the total weight of the solution, of the polymer in the solvent when the solution is to be used for the preparation of fibers and filaments, it is to be understood that as little as 5 percent or less and more than 50 percent of the polypyrrolidone may be dissolved in the solvents of this invention when the solution is to be employed for other purposes, such as a coating or a lacquer and the like, or when lower and higher molecular weight polymers are to be dissolved. The amount of any specific polymer which can be dissolved in the solvents of this invention will be readily evident to those skilled in the art.

The solvents of this invention readily dissolve polypyrrolidone within a wide range of temperature depending upon the nature of the polymer, the concentration thereof in the solvent and the nature of the solvent itself. Although temperatures within the range of 15° C. to 120° C. are preferred in bringing about the solution, temperatures as low as 5° C. and as high as the boiling point of the polymer/solvent mixture may be employed where necessary to bring about dissolution. Heating of the polymer/solvent mixture is preferably accomplished on a water, glycerine or oil bath. However, other means may be employed. If desired, agitation or stirring of the mixture may be employed during heating or when a solution is being formed at low temperatures, although it is to be understood that it is not always necessary or critical.

If it is desired to produce shaped articles from the polypyrrolidone compositions of the present invention which have a modified appearance and modified properties, various agents to accomplish these effects may be added to the polymer solutions prior to fabrication of the articles without having any ill effects thereon. Such added agents may be plasticizers, pigments, dyes, anti-static agents, fire-retarding agents, and the like.

The following examples are intended to illustrate the new compositions of this invention more fully but are not intended to limit the scope of the invention, for it is possible to effect many modifications therein. In the examples, all parts and percents are by weight unless otherwise indicated.

#### Example I

To a 25 gram (0.294 mole) sample of essentially anhydrous pyrrolidone, there was added under a nitrogen atmosphere 0.75 gram (0.0315 mole) of sodium hydride catalyst. When the evolution of hydrogen gas was completed, 0.56 gram (0.00295 mole) of titanium tetrachloride was added to the reaction mixture. This mixture was stoppered to protect it against the atmosphere and was permitted to stand for 25 hours at about 25° C. The polymer was recovered by breaking up the cake, grinding it in a Wiley mill, and washing the powder, first with water, then with acetone, in a Waring Blender. The polymer was subsequently air-dried to constant weight. The polymer had a specific viscosity of 0.761 (determined on 0.5 percent solutions of the polymer in 90 percent formic acid at 25° C.).

4.75 parts of phytic acid and 4.75 parts of water were

mixed and 0.50 part of the polypyrrolidone prepared above. The mixture was heated at 95° C. on a glycerine bath for 1½ hours with occasional stirring. The solution formed was clear, slightly viscous, and stable at 25° C. Fibers drawn therefrom were washed in 25 percent aqueous sodium hydroxide solution. These fibers were cold drawable and had good tensile strength. A clear film was made from the solution by dipping a glass rod, coated with the solution, into a bath containing 25 percent aqueous sodium hydroxide.

#### Example II

To a 25 gram (0.294 mole) sample of essentially anhydrous pyrrolidone, there was added under a nitrogen atmosphere 0.75 gram (0.0315 mole) of sodium hydride catalyst. When the evolution of hydrogen gas was completed, 0.39 gram (0.00293 mole) of anhydrous aluminum chloride was added to the reaction mixture. This mixture was stoppered to protect it against the atmosphere and permitted to stand for 25 hours at about 25° C. The polymer was recovered as in the foregoing example and had a specific viscosity, determined on 0.5 percent solutions of the polymer in 90 percent formic acid at 25° C., of 3.914.

Subsequently, 2.0 parts of the polypyrrolidone so prepared were mixed with 4.0 parts of phytic acid and 4.0 parts of water. This mixture was heated at 105° C. on a glycerine bath for 3½ hours with occasional stirring. The solution formed was clear, slightly viscous, and stable at 25° C. However, the mixture became somewhat cloudy at this temperature. Fibers drawn therefrom were washed in 25 percent sodium hydroxide solution. These fibers were cold drawable and had good tensile strength. A clear film was obtained from the solution by submersing a glass rod, coated with the solution into a bath containing 25 percent sodium hydroxide solution.

#### Example III

5.25 parts of phytic acid and 2.25 parts of water were mixed with 2.50 parts of the polypyrrolidone prepared in Example I. The mixture was heated on a glycerine bath at 105° C. for 1 hour. The solution formed was clear, viscous, and stable at 25° C. Fibers drawn therefrom were washed with a 15 percent aqueous sodium hydroxide solution. These fibers were cold drawable and had good tensile strength. A film was obtained from the solution by dipping a glass rod therein and thereafter submersing the rod covered with the solution in a bath containing 15 percent aqueous sodium hydroxide solution.

#### Example IV

To a 25 gram (0.294 mole) sample of essentially anhydrous pyrrolidone, there was added under a nitrogen atmosphere 0.75 gram (0.0315 mole) of sodium hydride catalyst. When the evolution of hydrogen gas was completed, 0.78 gram (0.00298 mole) of stannic chloride was added to the reaction mixture. This mixture was stoppered to protect it against the atmosphere and was permitted to stand for 25 hours at about 25° C. The polymer was recovered as in Example I and had a specific viscosity of 4.372, determined on 0.5 percent solutions of the polymer in 90 percent formic acid at 25° C.

6.65 parts of phytic acid and 2.85 parts of water were mixed with 0.50 part of the polypyrrolidone prepared by the procedure hereinabove. The mixture was heated on a glycerine bath at 60° C. for 45 minutes with occasional stirring. The solution formed was clear and slightly viscous. It was stable at 25° C. Fibers drawn therefrom were washed in 15 percent aqueous sodium hydroxide solution. These fibers were cold drawable and had good tensile strength. A film was made by dipping a glass rod covered with the solution into a bath containing 15 percent aqueous sodium hydroxide solution.

*Example V*

8.55 parts of phytic acid and 0.95 part of water were mixed with 0.50 part of the polypyrrolidone prepared in Example I. The mixture was heated on a glycerine bath at 90° C. for 1 hour. The solution was clear, slightly viscous and stable at temperatures of 25° C. Fibers drawn therefrom were washed in 15 percent aqueous sodium hydroxide solution. These fibers were cold drawable and had good tensile strength. A film was made by submersing a glass rod coated with the solution into a bath containing 15 percent aqueous sodium hydroxide solution. The film was clear and strong.

*Example VI*

To a 25 gram (0.294 mole) sample of essentially anhydrous pyrrolidone, there was added under a nitrogen atmosphere 0.75 gram (0.0315 mole) of sodium hydride catalyst. When the evolution of hydrogen gas was completed, 0.88 gram (0.00294 mole) of antimony pentachloride was added to the reaction mixture. The mixture was stoppered to protect it against the atmosphere and was permitted to stand for 25 hours at about 25° C. The polymer was recovered by the procedure disclosed in the foregoing examples and had a specific viscosity of 3.024, determined on 0.5 percent solutions of the polymer in 90 percent formic acid at 25° C.

4.75 parts of calcium acid phytate and 4.75 parts of water were mixed with 0.50 part of the polypyrrolidone prepared in accordance with the above procedure. The mixture was heated on a glycerine bath at 73° C. for 45 minutes with occasional stirring. The solution formed was clear, viscous, and stable at 25° C. Fibers drawn therefrom were washed in 15 percent aqueous sodium hydroxide solution. These fibers were cold drawable and had good tensile strength. A film was obtained by dipping a glass rod covered with the polymer solution into a bath containing 15 percent aqueous sodium hydroxide solution. The film was clear and had good strength.

*Example VII*

3.75 parts of calcium acid phytate and 3.75 parts of water were mixed with 2.50 parts of the polypyrrolidone prepared in accordance with the procedure of Example II. This mixture was heated on a glycerine bath at 107° C. for 1½ hours with occasional stirring. The solution formed was clear, viscous, and stable at 25° C. Fibers drawn therefrom were washed in 15 percent aqueous sodium hydroxide solution. These fibers were cold drawable and had good tensile strength. A clear film was made from the solution by dipping a glass rod coated therewith into a bath containing 15 percent aqueous sodium hydroxide solution. The film was clear and had good strength.

*Example VIII*

4.75 parts of calcium acid phytate and 4.75 parts of water were precooled to 5° C. and mixed with 0.50 part of the polypyrrolidone prepared in accordance with the procedure of Example II. The mixture went into solution with occasional stirring at a temperature in a range of 5 to 20° C. in 4 hours. The solution was clear, viscous, and stable at temperatures as low as 5° C. Fibers drawn therefrom were washed in 15 percent aqueous sodium hydroxide solution. These fibers were cold-drawable and had good tensile strength. A clear film was made by dipping a glass rod coated with the solution into a bath containing 15 percent aqueous sodium hydroxide solution.

*Example IX*

6.65 parts of phytic acid and 2.85 parts of water were precooled to 5° C. and mixed with 0.50 part of the poly-pyrrolidone prepared in accordance with the procedure of Example VI. The mixture went into solution with occasional stirring at a temperature in a range of 5 to 20° C.

in 4 hours. The solution was clear, viscous and stable at temperatures as low as 5° C. Fibers drawn therefrom were washed in 15 percent aqueous sodium hydroxide solution. These fibers were cold drawable and had good tensile strength. A clear film was made by dipping a glass rod coated with the solution into a bath containing 15 percent aqueous sodium hydroxide solution,

10 The new compositions of this invention present many advantages. For example, solutions of polypyrrolidone may be easily prepared on existing equipment without detailed and elaborate procedures. The phytic acid solvents of this invention are inexpensive and readily available. Furthermore, the new solvents of this invention are entirely harmless, since they are neither toxic nor explosive and, therefore, may be employed without extraordinary precaution. Polymeric solutions made with the new solvents of this invention are clear and colorless, and products or shaped articles prepared from such solutions exhibit superior color characteristics. In addition 15 to these advantages, the solvents of this invention are further advantageous in that they have no effect upon the desirable chemical and physical properties of the polymers dissolved therein. Numerous other advantages of the new compositions of this invention will be readily apparent to those skilled in the art.

It will be understood to those skilled in the art that many apparently widely different embodiments of this invention can be made without departing from the spirit and scope thereof. Accordingly, it is to be understood that this invention is not to be limited to the specific embodiments thereof except as defined in the appended claims.

I claim:

1. A new composition of matter comprising polypyrrrolidone dissolved in a solvent containing 5 to 50 percent by weight of water, based on the total weight of the solvent, and 95 to 50 percent of a compound selected from the group consisting of phytic acid, the water-soluble alkali metal acid salts of phytic acid, the alkaline earth metal acid salts of phytic acid, and the mixed alkali and alkaline earth metal acid salts of phytic acid.

2. A new composition of matter as defined in claim 1 wherein the solvent contains phytic acid.

3. A new composition of matter as defined in claim 1 wherein the solvent contains calcium acid phytate.

4. A new composition of matter as defined in claim 1 wherein the solvent contains sodium acid phytate.

5. A new composition of matter as defined in claim 1 wherein the solvent contains magnesium acid phytate.

6. A new composition of matter as defined in claim 1 wherein the solvent contains potassium acid phytate.

7. A new composition of matter comprising 5 to 50 percent, based on the total weight of the composition, of polypyrrrolidone dissolved in a solvent containing 5 to 50 percent by weight of water, based on the total weight of the solvent, and 95 to 50 percent of a compound selected from the group consisting of phytic acid, the water-soluble alkali metal acid salts of phytic acid, the alkaline earth metal acid salts of phytic acid, and the mixed alkali and alkaline earth metal acid salts of phytic acid.

8. A new fiber-forming composition of matter comprising 20 to 40 percent, based on the total weight of the composition, of polypyrrrolidone, having a specific viscosity of at least 0.3, dissolved in a solvent containing 30 to 50 percent by weight of water, based on the total weight of the solvent, and 70 to 50 percent of a compound selected from the group consisting of phytic acid, the water-soluble alkali metal acid salts of phytic acid, the alkaline earth metal acid salts of phytic acid, and the mixed alkali and alkaline earth metal acid salts of phytic acid.

9. A process for preparing a new composition of matter comprising mixing polypyrrrolidone and a solvent containing 5 to 50 percent by weight of water, based on

75

the total weight of the solvent, and 95 to 50 percent of a compound selected from the group consisting of phytic acid, the water-soluble alkali metal acid salts of phytic acid, the alkaline earth metal acid salts of phytic acid, and the mixed alkali and alkaline earth metal acid salts of phytic acid, and subjecting the mixture to a temperature in a range of 5° C. to the boiling point of the mixture to form a homogeneous solution.

10. The process as defined in claim 9 wherein the solvent contains phytic acid.

11. The process as defined in claim 9 wherein the solvent contains calcium acid phytate.

12. The process as defined in claim 9 wherein the solvent contains sodium acid phytate.

13. The process as defined in claim 9 wherein the solvent contains magnesium acid phytate.

14. The process as defined in claim 9 wherein the solvent contains potassium acid phytate.

15. A process for preparing a new fiber-forming composition of matter comprising mixing 30 percent, based on the total weight of the composition, of poly-pyrrolidone, having a specific viscosity of 3.914, and a solvent containing 50 percent of phytic acid and 50 percent of water, based on the total weight of the solvent, and heating the mixture to a temperature of 107° C. to form a homogeneous solution.

References Cited in the file of this patent

UNITED STATES PATENTS

15 2,638,463 Ney et al. May 12, 1953  
2,734,004 Robinson Feb. 7, 1956